

1

3,510,431

### HIGH TEMPERATURE SYNTHETIC ESTER BASE LUBRICANT COMPOSITION BLENDS WITH LIQUID DIESTERS OF DIHYDROXY BIPHENYLS

Tai S. Chao, Homewood, Ill., and Manley Kjonaas, Hammond, Ind., assignors to Sinclair Research, Inc., New York, N.Y., a corporation of Delaware  
No Drawing. Filed Aug. 24, 1967, Ser. No. 662,902  
Int. Cl. C10m 3/20

U.S. CL. 252—57

9 Claims

#### ABSTRACT OF THE DISCLOSURE

Esters of certain branched chain fatty acids containing a quaternary carbon atom and dihydroxy biphenyls are employed as base fluids or blending stock in lubricants. Lubricants containing these esters possess suitable viscosity characteristics and greater thermal and oxidative stability and are of special value in lubricating engines which are subject to high temperatures.

This invention is concerned with liquid synthetic esters which are suitable, for instance, for use as base fluids in lubricants.

Lubricants composed in whole or in part of synthetic components have been developed in an effort to obtain superior lubricating compositions. In general, these lubricating compositions are characterized by higher viscosity index, lower pour point and greater heat stability than mineral oils of corresponding viscosity. Such properties are of special value in lubricating engines which are subjected to high temperatures, such as combustion turbine engines. Mineral oil lubricants, even those containing added VI improvers, pour point depressors, or other additives are undesirable for use in such engines because of the relatively high volatility, low flash point and poor thermal and oxidative stability of the mineral oils, which also have a tendency to leave deposits which accumulate and interfere with the operation of the engine. Particularly, in high performance jet engines, such as those designed for supersonic transport and other advanced aircraft, and in industrial gas turbines which operate continuously at full power settings, lubricants are required to have high thermal and oxidative stability.

Certain neoalkylpolyol esters of straight chain fatty acids, e.g., pentaerythritol tetracaproate, which are known as Type II lubricants, have been employed in jet engines but do not possess the thermal and oxidative stability required of the more advanced engine models. On the other hand, esters derived from neoalkylpolyols and branched-chain fatty acids, e.g., pentaerythritol tetrapivalate, although having good oxidative stability, are solids at room temperatures and thus have poor handling, starting and low temperature properties. Polyphenyl ethers, e.g., m,m',m-bisphenoxyphenoxybenzene, have pour points above 35–40° F. and do not flow and pour at subzero temperatures, as required to achieve their functions, especially during the critical start up time for jet engines.

It has now been found that the esters formed by reacting certain branched chain fatty acids or acid chlorides containing a quaternary carbon atom with dihydroxy biphenyls possess superior properties of thermal and oxidative stability along with suitable viscosity, volatility and low temperature properties and therefore may be employed as either base fluids or blending stocks in lubricants for high performance supersonic aircraft and other gas turbine engines. In addition these esters can be used as base fluids or thickeners for high temperature hydraulic fluids, base fluids for high temperature greases and as components for other lubricants which require high thermal and oxidative stability. They can also be used as ad-

2

vanced plasticizers for high temperature polymers such as polyvinyl chloride, polyethylene, polyesters, polyamides, polyimides, polycarbonates, synthetic rubber, etc.

Aromatic dihydroxy biphenyls suitable for forming the esters of this invention may be described by the general formula:



wherein  $x$  equals 0–2,  $y$  equals 0–2, and  $x+y$  equal 2–4. The aromatic rings of these dihydroxy biphenyls may be further substituted with non-deleterious organic groups, especially those of up to about four carbon atoms, such as the lower alkyls and lower alkoxy.

Suitable dihydroxy-biphenyls include 2,2'-dihydroxy biphenyl, 4,4'-dihydroxy biphenyl, 2,4-dihydroxy biphenyl, 2,4'-dihydroxy biphenyl, 3,3'-dihydroxy biphenyl, 2,2'-dihydroxy-4,4'-dimethyl biphenyl, 2,2'-dihydroxy-4,4'-dimethoxy biphenyl, 4,4'-dihydroxy-3,3',5,5'-tetramethyl biphenyl, etc. These compounds are readily prepared by the oxidative coupling of the corresponding monohydric phenols. For example, 2,2'-dihydroxy-4,4'-dimethyl biphenyl is obtained when p-cresol is oxidized in the presence of  $\text{FeCl}_3$  (Bowden & Reece, J. Chem. Soc. 1950, 2249).

The fatty acid chlorides are prepared by reacting appropriate fatty acids with compounds such as  $\text{PCl}_3$ ,  $\text{PCl}_5$ ,  $\text{SOCl}_2$ . These fatty acids have the general structure:



wherein  $m$  is 0 to 3 and  $\text{R}_1$ ,  $\text{R}_2$  and  $\text{R}_3$  are alkyl groups having 1 to 4 carbons. Exemplary of these acids are the following acids which can be used separately or as mixtures thereof to produce the esters of this invention: 2,2-dimethylpentanoic acid, 3,3-dimethylpentanoic acid, 4,4-dimethylpentanoic acid, 4,4-dimethylhexanoic acid, 3,3,4-trimethylpentanoic acid, 4,4,5-trimethylhexanoic acid, 3,3-dimethylbutanoic acid, 2-methyl-2-ethyl pentanoic acid, 3-methyl-3-ethyl pentanoic acid, 3-methyl-3-ethyl butanoic acid, neo-octanoic acid (mixture of  $\text{C}_8$  acids having neo acid structures), and neodecanoic acid.

The esterification reaction with the dihydroxy biphenyl can be carried out using either the fatty acid directly or using the acid chloride. In the event the fatty acid is reacted directly with the aromatic hydroxy compound a suitable reagent such as trifluoroacetic anhydride or polyphosphoric acid can also be employed to combine with the water of reaction. If the acid chloride is employed rather than the acid, the reaction is facilitated by the presence of a compound which will react with the  $\text{HCl}$  as it is formed. Such  $\text{HCl}$  acceptors include certain amines which have no hydrogen on the nitrogen atom, such as pyridine, dimethyl aniline, and triethylamine, and also inorganic bases such as  $\text{Na}_2\text{CO}_3$  and  $\text{CaCO}_3$ . The  $\text{HCl}$  may also be removed from the reacting mixture by applying sufficient heat and bubbling nitrogen through it. Suitable solvents such as benzene, toluene, xylene, chloroform and ether may be employed to facilitate the reaction and to make stirring easier. The rate of the reaction is increased by the use of a catalyst such as dimethyl formamide.

An illustration of the esterification is given in the example.

#### EXAMPLE

2,2'-bis(2,2-dimethylpentanoxy)biphenyl was prepared in the following manner:

A mixture of 186 g. (1.0 mole) of 2,2'-dihydroxy bi-

phenyl (also called O,O'-biphenol) and 400 g. of toluene was refluxed in a 3 liter, 4-neck flask equipped with a Dean-Stark trap to remove a trace of water. The solution was cooled to about 80° C. when 15 ml. of dimethylformamide was added. With constant stirring and keeping the mixture in the flask at 76°-82° C., 328 g. (2.2 moles) of neoheptanoyl chloride was added during a period of 4.5 hours. Vivid evolution of HCl gas was observed. The mixture was stirred at 80°-100° C. for 6 hours. After the addition of 30 ml. of pyridine, the mixture was further stirred (at 90°-100°) for 6 hours. Upon cooling, it was washed twice with dilute HCl, twice with 10% NaOH and twice with water. The solution was then topped to 180°/1 mm., yielding 400 g. of light colored liquid. The light colored liquid was distilled at 187°-192° pot temperature and 0.15 to 0.20 mm. Hg to give an almost colorless liquid having a kinematic viscosity at 210° F. of 6.164 cs. and pour point of -20° F.

Using the general procedure described in the example, any of the dihydroxy biphenyls named herein can be reacted with any of the fatty acids named herein or their corresponding acid chlorides to give the esters of this invention. Thus 4,4'-bis(2,2-dimethylpentanoyloxy)biphenyl is obtained by reacting 4,4'-dihydroxy biphenyl with 2,2-dimethylpentanoyl chloride or 2,2-dimethylpentanoic acid. In the same manner 2,2'-bis(3,3-dimethylpentanoyloxy)biphenyl is obtained by reacting 2,2'-dihydroxybiphenyl with 3,3-dimethylpentanoyl chloride or 3,3-dimethylpentanoic acid. Using 2,4-dihydroxy biphenyl and 2,2-dimethylpentanoic acid, there is obtained 2,4-bis(2,2-dimethylpentanoyloxy)biphenyl. 2,2'-dihydroxy-4,4'-dimethoxy biphenyl with 3,3-dimethylpentanoic acid gives 2,2'-bis(3,3-dimethylpentanoyloxy)-4,4'-dimethoxybiphenyl. 4,4'-dihydroxy-3,3',5,5'-tetramethyl biphenyl with 4,4-dimethylhexanoic acid gives 4,4'-bis(4,4'-dimethylhexanoyloxy)-3,3',5,5'-tetramethyl biphenyl.

The esters produced by the process of this invention are diacyloxybiphenyl compounds having the following structure:



where R<sub>1</sub>, R<sub>2</sub>, R<sub>3</sub>, x and y are the same as defined hereinbefore, m and n are 0-3, and each of the aromatic rings may be substituted with non-deleterious organic groups, especially those of up to about four carbon atoms such as lower alkyls and lower alkoxy.

It has also been found that the esters of this invention may be blended with other suitable esters to produce lubricating compositions having improved thermal and oxidative stability. Typical of the esters which may advantageously be blended with the esters of this invention are normal, neo, and gem alkanoic fatty esters of branched chain alcohols having 4 to 12 carbons and 2-6 OH's, e.g., esters of branched chain aliphatic alcohols, pentaerythritol, dipentaerythritol, trimethylol propane, neopentyl glycol, and fatty acids or mixtures thereof having 4-10 carbons, dibasic acid esters of monohydric aliphatic alcohols having 6 to 13 carbons and aliphatic acids of 6 to 12 carbons, and esters of dihydric phenols and fatty acids. These esters may be blended with the esters of the invention in amounts of from about 10 to 90% based on the weight of the lubricant. Examples of these blends of esters are found in Table III. Base fluids containing the esters of this invention have been found to possess improved oxidation resistance compared with conventional base fluids used as high temperature lubricants.

Oxidation resistance of the esters can be determined by the Oxygen Absorption Test which measures the rate of oxygen absorption in the presence of an inhibitor such as 1% N-phenyl-alpha-naphthylamine. The Oxygen Absorption Test is carried out in the following manner: a 75 gm. sample of the ester containing a standard anti-

oxidant is oxidized at 450° F. with 1 ft.<sup>3</sup>/hr. of oxygen in a tube of about 9" long and 1 1/4" in I.D. The exit gas passes through a reflux condenser, an entrainment trap and two absorption tubes. The first tube is filled with active charcoal, Drierite and Ascarite to remove organic vapor, water and CO<sub>2</sub>. The gases come out from the first tube then pass through a catalytic oxidation tube filled with CuO, in which CO and hydrocarbons are converted to CO<sub>2</sub>. The exit gas from the oxidation tube then passes through a second absorption tube filled with Drierite and Ascarite and is circulated with a tubing pump back into the sample tube. Thus oxygen is continuously circulated through the system until it is used up by the sample. The decrease in the volume of oxygen in the system which represents the volume of O<sub>2</sub> absorbed is continuously measured by a Statham gauge and recorded on a Brown recorder. The recorder is so calibrated that the slope of the curve represents the rate of oxygen absorption. During the earlier part of the test the oil is effectively inhibited by the antioxidant and the rate of O<sub>2</sub> absorption is usually small. The rate usually stays constant until a time is reached at which the inhibitor is either exhausted or is no longer effective in inhibiting the oxidation. At this point there is generally a fast increase in the rate of oxidation. The time in minutes required for this change of rate to take place is called induction time (T<sub>i</sub>). The volume of O<sub>2</sub> absorbed during this period of time is represented by V<sub>i</sub>. The test is continued until a total of 2500 ml. of O<sub>2</sub> has been absorbed. The time in minutes for this to take place is called total time (T<sub>t</sub>). The total volume of O<sub>2</sub> absorbed (V<sub>t</sub>) is usually 2500 ml., unless some other T<sub>t</sub> was used for special reasons.

Two conventional base fluids, pentaerythritol tetra-caproate and trimethylolpropane triheptanoate, were subjected to the Oxygen Absorption Test along with esters of this invention. The results are summarized in Table I.

TABLE I.—OXIDATION RESISTANCE OF ESTERS OF THIS INVENTION AS COMPARED TO THOSE OF CONVENTIONAL ESTERS

| Base fluid                                 | Test Temperature=450° F.<br>Antioxidant=1% N-phenyl-alpha-naphthylamine<br>Rate of O <sub>2</sub> =1 ft. <sup>3</sup> /hr. |                        |                       |                       |
|--------------------------------------------|----------------------------------------------------------------------------------------------------------------------------|------------------------|-----------------------|-----------------------|
|                                            | T <sub>i</sub><br>min.                                                                                                     | T <sub>t</sub><br>min. | V <sub>i</sub><br>ml. | V <sub>t</sub><br>ml. |
| Trimethylolpropane triheptanoate           | 239                                                                                                                        | 278                    | 614                   | 2,500                 |
| Pentaerythritol tetraheptanoate            | 260                                                                                                                        | 298                    | 474                   | 2,500                 |
| 4,4'-bis(2,2-dimethylpentanoyloxy)biphenyl | 906                                                                                                                        | 906                    | -----                 | 2,500                 |
| 2,2'-bis(2,2-dimethylpentanoyloxy)biphenyl | 1,928                                                                                                                      | 1,928                  | -----                 | 2,500                 |
| 2,2'-bis(3,3-dimethylpentanoyloxy)biphenyl | 1,493                                                                                                                      | 1,493                  | -----                 | 2,500                 |

50

As may be seen in Table I, the esters containing the biphenyl groups have induction times (T<sub>i</sub>) and total times (T<sub>t</sub>) 3 to 6 times greater than the two conventional base fluids tested which are often present in Type II synthetic lubricants. This much greater period of time required for the esters of this invention to absorb 2500 ml. of O<sub>2</sub> is indicative of the improved resistance to oxidation which will result. Lubricants containing these esters as base fluids will therefore last longer in gas turbine engines, and form less troublesome oxidation products such as sludge, coke and acids. It is further seen in Table II that there is no sacrifice in desirable properties of viscosity, pour, flash, and fire points found in the compounds.

| Kinematic viscosity: | 2,2'-bis(2,2-dimethylpentanoyloxy)biphenyl | 4,4'-bis(2,2-dimethylpentanoyloxy)biphenyl | 2,2'-bis(3,3-dimethylpentanoyloxy)biphenyl |
|----------------------|--------------------------------------------|--------------------------------------------|--------------------------------------------|
| 210° F.              | 6.164                                      | 14.6                                       | 8.778                                      |
| 100° F.              | 82.20                                      | 313.9                                      | 174.1                                      |
| Pour point, ° F.     | -20                                        | 940                                        | -15                                        |
| Flash point, ° F.    | 405                                        | 0                                          | 445                                        |
| Fire point, ° F.     | 470                                        | -----                                      | 515                                        |

70

75

TABLE III

| 50 wt. percent<br>4,4'-bis(2,2'-<br>dimethylpen-<br>tanoxyloxy)<br>biphenyl, 50 wt.<br>percent resor-<br>cinol dineo-<br>ctanoate | 70 wt. percent<br>2,2'-bis(2,2'-<br>dimethylpen-<br>tanoxyloxy)<br>biphenyl, 30 wt.<br>percent di-<br>pentaerythritol<br>ester of valeric<br>and neohep-<br>tanoic acids | 50 wt. percent<br>2,2'-bis(3,3'-<br>dimethylpen-<br>tanoxyloxy)-<br>biphenyl, 50 wt.<br>percent pent-<br>aerythritol<br>ester of valeric<br>and neohep-<br>tanoic acids |
|-----------------------------------------------------------------------------------------------------------------------------------|--------------------------------------------------------------------------------------------------------------------------------------------------------------------------|-------------------------------------------------------------------------------------------------------------------------------------------------------------------------|
| Kinematic viscosity, cs.:                                                                                                         |                                                                                                                                                                          |                                                                                                                                                                         |
| 210° F.-----                                                                                                                      | 7.910                                                                                                                                                                    | 7.244                                                                                                                                                                   |
| 100° F.-----                                                                                                                      | 105.3                                                                                                                                                                    | 84.99                                                                                                                                                                   |
| 0° F.-----                                                                                                                        | 60.719                                                                                                                                                                   | 36.211                                                                                                                                                                  |
| Pour point, ° F.-----                                                                                                             | -30                                                                                                                                                                      | -30                                                                                                                                                                     |
| Cloud point, ° F.-----                                                                                                            | below -30                                                                                                                                                                | below -30                                                                                                                                                               |
| Flash point, ° F.-----                                                                                                            | 440                                                                                                                                                                      | 420                                                                                                                                                                     |
| Fire point, ° F.-----                                                                                                             | 505                                                                                                                                                                      | 490                                                                                                                                                                     |
|                                                                                                                                   |                                                                                                                                                                          | 510 15                                                                                                                                                                  |

It is claimed:

1. A high temperature synthetic ester base lubricant composition consisting essentially of a blend of:  
(A) from about 10 to 90 weight percent of a liquid diester of (a) a dihydroxy biphenyl of the formula



wherein  $x$  and  $y=0-2$  but  $x+y=2$  and (b) a branched chain acid having a quaternary carbon atom selected from the group consisting of: 2,2-dimethylpentanoic acid, 3,3-dimethylpentanoic acid, 4,4-dimethylpentanoic acid, 4,4-dimethylhexanoic acid, 3,3,4-trimethylpentanoic acid, 4,4,5-trimethylhexanoic acid, 3,3-dimethylbutanoic acid, 2-methyl-2-ethyl pentanoic acid, 3-methyl-3-ethyl pentanoic acid, and 3-methyl-3-ethyl butanoic acid, and

(B) from about 90 to 10 weight percent of an ester selected from the group consisting of (a) the normal, neo and gem alkanoic fatty acid esters of branched chain aliphatic alcohols having 4 to 12 carbons and 2 to 6 hydroxy groups and alkanoic fatty acids having 4 to 10 carbons and mixtures thereof, (b) dibasic acid esters of monohydric aliphatic alcohols having 6 to 13 carbons and aliphatic acids of 6 to 12 carbons, and (c) esters of dihydric phenols and fatty acids.

2. A high temperature synthetic ester base lubricant composition consisting essentially of a blend as set forth in claim 1 wherein said liquid diester of a dihydroxy diphenyl (A) is 2,2'-bis(2,2-dimethylpentanoxyloxy)biphenyl and said ester (B) is the dipentaerythritol ester of a mixture of valeric and neoheptanoic acids.

3. A high temperature synthetic ester base lubricant composition consisting essentially of a blend as set forth in claim 2 wherein said 2,2'-bis(2,2-dimethylpentanoxyloxy)biphenyl is 70 weight percent and said dipentaerythritolester of a mixture of valeric and neoheptanoic acids is 30 weight percent.

4. A high temperature synthetic ester base lubricant composition consisting essentially of a blend as set forth in claim 1 wherein said liquid diester of a dihydroxy

biphenyl (A) is 4,4'-bis(2,2-dimethylpentanoxyloxy)biphenyl and said ester (B) is resorcinol dineooctanoate.

5. A high temperature synthetic ester base lubricant composition consisting essentially of a blend as set forth in claim 4 wherein said 4,4'-bis(2,2-dimethylpentanoxyloxy)biphenyl is 50 weight percent and said resorcinol dineooctanoate is 50 weight percent.

6. A high temperature synthetic ester base lubricant composition consisting essentially of a blend as set forth in claim 1 wherein said liquid diester of a dihydroxy biphenyl (A) is 2,2'-bis(3,3-dimethylpentanoxyloxy)biphenyl and said ester (B) is the pentaerythritol ester of a mixture of valeric and neoheptanoic acids.

7. A high temperature synthetic ester base lubricant composition consisting essentially of a blend as set forth in claim 6 wherein said 2,2'-bis(3,3-dimethylpentanoxyloxy)biphenyl is 50 weight percent and said pentaerythritol ester of a mixture of valeric and neoheptanoic acids is 50 weight percent.

8. A high temperature synthetic ester base lubricant composition consisting essentially of a blend of:

(A) from about 10 to 90 weight percent of a liquid diester of (a) a dihydroxy biphenyl of the formula



wherein  $x$  and  $y=0-2$  but  $x+y=2$  and (b) a branched chain acid having a quaternary carbon atom selected from the group consisting of: 2,2-dimethylpentanoic acid, 3,3-dimethylpentanoic acid, and 4,4-dimethylpentanoic acid, and

(B) from about 90 to 10 weight percent of an ester selected from the group consisting of (a) the normal, neo and gem alkanoic fatty acid esters of branched chain aliphatic alcohols having 4 to 12 carbons and 2 to 6 hydroxy groups and alkanoic fatty acids having 4 to 10 carbons and mixtures thereof, (b) dibasic acid esters of monohydric aliphatic alcohols having 6 to 13 carbons and aliphatic acids of 6 to 12 carbons, and (c) esters of dihydric phenols and fatty acids.

9. A high temperature synthetic ester base lubricant composition consisting essentially of a blend as set forth in claim 8 wherein said dihydroxy biphenyl is 2,2'-dihydroxy biphenyl or 4,4'-dihydroxy biphenyl.

#### References Cited

##### UNITED STATES PATENTS

- 2,961,406 11/1960 McNeil.  
3,309,318 3/1967 Aylesworth et al.  
3,347,884 10/1967 Voris 252-57

##### FOREIGN PATENTS

- 855,242 11/1960 Great Britain.

##### OTHER REFERENCES

- R. S. Barnes et al.: "Synthetic Ester Lubricants," Lubrication Engineering, August 1957, 454-458.

DANIEL E. WYMAN, Primary Examiner

J. M. HICKEY, Assistant Examiner

UNITED STATES PATENT OFFICE  
CERTIFICATE OF CORRECTION

Patent No. 3,510,431 Dated May 5, 1970

Inventor(s) Tai S. Chao and Manley Kjonaas

It is certified that error appears in the above-identified patent and that said Letters Patent are hereby corrected as shown below:

In the formula which appears in Column 2, Line 32,

"—C—" should be --—C—--.  
  III                            II  
  0                            0

In Column 4, Table I, "T<sub>1</sub>" should read --T<sub>t</sub>--.

In Column 4, Table II, "940" should read --0--, and "0" should read --490--.

In Column 5, Table III, the right hand column of Table III, "valerie" should read --valeric--.

In Column 5, Table III, the next to the right hand column "84.99" should read --84.89--.

**SIGNED AND  
SEALED  
OCT 13 1970**

**(SEAL)**

**Attest:**

**Edward M. Fletcher, Jr.**

**Attesting Officer**

**WILLIAM E. SCHUYLER, JR.**  
Commissioner of Patents